

2,962,440

## PRODUCTION OF A SMOOTH, UNIFORM, AIR-FREE ALUMINUM STEARATE GREASE

John Francis Richards and Russell Albert Thompson, Jr.,  
Baton Rouge, La., assignors to Esso Research and Engineering Company, a corporation of Delaware

No Drawing. Filed Oct. 27, 1958, Ser. No. 769,564

4 Claims. (Cl. 252—35)

This invention relates to a new process for producing a smooth, uniform, air-free aluminum stearate grease which involves the addition of a portion of the blending oil to a base concentrate grease under vacuum.

There are, at present, two main methods of making and processing an aluminum stearate grease. In one the grease is packaged when hot and molten and upon cooling a "gel" forms. This "gel" is of a rubbery consistency of such a nature as to actually bounce back a hard article that might be poked at it and is distinguishable from a normal grease structure. The disadvantage of this first technique is that the hardness of the "gel" which forms on cooling varies with the cooling rate. The differing cooling rates experienced in different size containers and even in different parts of the same container cause the grease to vary in consistency. Even samples taken from the grease kettle have different cooling rates and consistencies from the final packaged product. Since control samples taken from the kettle do not give the same consistency as the same grease will eventually have in the container, it is very difficult to adjust the grease in the kettle so as to get the desired consistency in the container. Also a waiting period of about 48 hours to complete cooling and gel formation is necessary before samples from the package can be tested to see if they meet consistency specifications.

The other main method of commercially producing aluminum stearate grease allows the hot, molten grease to be run into pans, air cooled to room temperature, dumped back into the kettle, stirred to break the "gel" without heating and then cutback to the desired consistency with oil. The pan cooled grease is a concentrate so that anyone of several different thickness greases can be made by varying the cutback proportions. While a uniform product can be obtained by this latter method, it is very time consuming, laborious and requires extreme care to prevent aerating the grease since the grease is stirred while cold and any entrapped air will not easily work out of the solid grease.

The present invention now obviates the difficulties of the two aforementioned commercial procedures, since now the rubbery "gel" is broken up as the grease is initially prepared in the kettle. In this way no "gel" is formed after the grease is packaged as happens in the first method and the advantage of control of final consistency which is a valuable part of the second process is retained without time consuming and excess steps.

The method of the present invention involves cooling an aluminum stearate grease concentrate under vacuum and simultaneously adding the balance of the constituent oil as a coolant. Only one sample for adjustment need be taken after cooling to a temperature of 120° F. or less. The grease may then be packaged at 120° F. or less directly from the kettle. The waiting and sampling occasioned by the non-uniform product of the other processes are now not necessary. There is no guess work involved in adjusting consistency since the grease is cooled and

the "gel" broken before sampling, by the action of the kettle paddles.

The term aluminum stearate as used in this specification and claims includes not only the pure aluminum mono-, di-, and tri-stearates and mixtures thereof in any proportion, but also includes commercial aluminum stearates. The commercial aluminum stearates are generally mixtures of the mono-, di-, and tri-soaps. The soap itself, while generally predominately stearate, may also contain minor quantities of the soaps of C<sub>14</sub> to C<sub>22</sub> fatty acids, particularly the C<sub>14</sub> and C<sub>16</sub> acids. Thus, a typical "hi-gel" aluminum stearate will consist of about 2/3 of the di-soap and about 1/3 of the mono-soap. This mono- and di-soap will be about 55-85% stearate, with substantial amounts of palmitate and lesser amounts of other fatty acids. A "low gel" stearate or "oil type" stearate will comprise about 2/3 of the mono-soap and about 1/3 of the di-soap. The mono- and di-soaps again being mixtures of soaps of various fatty acids as described above.

The lubricating greases of the invention will comprise about 1 to 7, but preferably 2.5 to 5.0 parts by weight of aluminum stearate per 100 parts by weight of mineral lubricating oil.

Various other additives may also be added to the lubricating composition in amounts of about 2 to 4 but preferably 2.4 to 2.5 weight percent, based on the total weight of the composition. Examples of such additives include: oxidation inhibitors such as phenyl-alpha-naphthylamine; corrosion inhibitors such as sorbitan monoleate; dyes; other grease thickeners and the like.

The technique of this invention consists of heating the soap in a portion of the oil to obtain a dispersion. Generally the soap and oil is heated to about 250° to 450° F., e.g. 280° to 350° F. in about 25 to 75, preferably 30 to 35 weight percent of the total oil for about 2 to 4 hours or until the solids dissolve. The kettle is then closed and put under a vacuum so that the absolute pressure in the kettle is about 0 to 7.7 p.s.i.a. Cooling water is put through the kettle jacket and the balance of the oil is added to the kettle without affecting the vacuum. Cooling is continued until the grease is 120° F. or less. The batch is sampled, and the consistency ascertained. Finally, after making any necessary adjustments to the consistency, the grease is packaged at a temperature of 120° F. or less. Adding the remaining portion of the oil while cooling also helps shorten the cooling cycle. The vacuum prevents aeration and the action of the kettle paddles breaks up any "gel" as it might form in the kettle thus resulting in a uniform product.

The invention will be further understood by the following example:

Example I (all parts by weight)

31 parts by weight of a mineral lubricating oil having a viscosity of 120-130 SUS. at 210° F., 4.4 parts by weight of a commercial aluminum stearate (Plymouth-Parsons' No. 551) along with 2.4 parts by weight of an additive mixture consisting of 1.0 part oleic acid, 0.4 part aluminum naphthenate, and 1.0 part Paratac (polyisobutylene) were mixed together in the kettle while heating to a temperature of 250-300° F., which is sufficient to dissolve the solid stearate of the composition. The kettle was then closed and put under 6 p.s.i.a. Cooling water was run through the kettle jacket. Then the remainder of the lubricating oil, or about 62.2 parts by weight was added through a displacement meter. The composition was then cooled to 120° F. or less and sampled and tested for consistency. Further cooling to room temperature showed that no further change in consistency occurred. The resulting composition was an excellent

looking, clear, almost transparent grease with a smooth texture. Subsequent tests showed the grease was of uniform consistency, free of "gel" and air-free.

As a further illustration of my invention, Example I may be repeated, but using an aluminum soap consisting of  $\frac{1}{3}$  aluminum monostearate and  $\frac{2}{3}$  aluminum distearate and omitting the additive mixture and heating to a maximum temperature of 300° F. before cooling.

In sum, the present invention comprises a method of producing an aluminum-stearate-oil composition while stirring under vacuum and cooling to a temperature of 120° F. or less. In this way the "gel" which tends to set up at a temperature of about 130° F. is broken up by the mixing action, and at the same time the presence of the vacuum prevents the entrapment of air in the grease while stirring at these low temperatures, i.e., about 120° F. The rate of cooling or length of time in adding the remainder of the lubricating oil does not have any effect on the process, but rather the critical features are in cooling to at least 120° F. while stirring under vacuum.

What is claimed is:

1. A method for producing a smooth, uniform, air-free aluminum stearate grease comprising about 1 to 7 parts by weight aluminum stearate and about 100 parts by weight of mineral lubricating oil which comprises forming a dispersion of said aluminum stearate in about 25 to 75 wt. percent of the total oil by heating to a temperature of about 250° to 450° F., cooling said dispersion to a temperature of less than about 120° F. under an

absolute pressure of about 0 to 7.7 p.s.i.a. while stirring and adding the balance of said oil, then packaging said grease.

2. A method according to claim 1, wherein said aluminum stearate is a mixture of mono-, di-, and tri-stearates.

3. A method according to claim 1, wherein said aluminum stearate is a commercial aluminum stearate, comprising about 55 to 85 wt. percent of stearate with minor amounts of aluminum soaps of C<sub>14</sub>—C<sub>22</sub> fatty acids.

4. A method for producing a smooth, uniform, air-free aluminum stearate grease comprising about 2.5 to 5.0 parts by weight of aluminum stearate and about 100 parts by weight of mineral lubricating oil, which comprises forming a dispersion of said aluminum stearate in about 30 to 35 wt. percent of the total oil by heating a mixture of said stearate in oil to about 280° to 350° F., placing the stearate-oil mixture under a reduced pressure of 0 to 7.7 p.s.i.a., adding the balance of said oil while stirring and cooling under said reduced pressure to a temperature less than 120° F.

References Cited in the file of this patent

UNITED STATES PATENTS

2,458,034 Swenson et al. \_\_\_\_\_ Jan. 4, 1949

OTHER REFERENCES

"The Manufacture and Application of Lubricating Greases," Boner, Reinhold Pub. Corp., N.Y., 1954, pp. 309 and 312.